# EUROPEAN PATENT SPECIFICATION

(11) **EP 0 783 598 B1**
(45) Date of publication and mention of the grant of the patent: **03.03.1999**
(21) Application number: 96925681.7
(22) Date of filing: 08.07.1996
(51) Int. Cl.: C25D 3/10

(54) **POLYCHROMATE CHROMIUM-PLATING PROCESS AND BATH**
VERFAHREN ZUR ABSCHEIDUNG VON CHROM AUS POLYCHROMAT-BÄDERN
PROCEDE DE CHROMAGE ET BAIN DE CHROMAGE CONTENANT DES POLYCHROMATES

(30) Priority: 28.07.1995 EP 95830339
(43) Date of publication of application: 16.07.1997
(73) Proprietor: LUIGI STOPPANI S.p.A., 20123 Milan (IT)
(72) Inventor: MERELLO, Giovanni, I-16155 Pegli (GE) (IT); FREDIANI, Lido, I-28100 Novara (IT)
(74) Representative: Gislon, Gabriele
(86) International application number: EP9602983
(87) International publication number: WO9705301

(56) References cited:
- CH-A- 673 845
- METAL FINISHING, vol. 65, no. 12, December 1967, USA, pages 63-70, XP000608389 DOMINIKOV: "chromium plating from polychromate bath"

## Description

### Technical Field

This invention relates to a process and a bath for chromium-plating by electrodeposition from a polychromate-based solution.

### Background Art

Polychromate-based chromium-plating baths have been known since 1933. They are usually prepared by mixing chromium anhydride and sodium hydroxide in solution.

A characteristic of polychromate-based chromium-plating baths is that they use high current densities and maintain high cathode efficiencies - 30% or more.

As well as this advantageous characteristic, polychromate-based chromium plating baths have a number of disadvantages which have limited their use on an industrial scale.

The deposit obtained is dull and has low covering power; it is difficult to prepare the polychromate-based chromium-plating baths on an industrial scale and, usually, the temperature of the bath must not exceed 20°C. Chromic-acid based chromium-plating baths are normally used to give brighter deposits, but these give low cathode efficiencies.

### Disclosure of the Invention

It is the object of the present invention to solve the aforementioned problems and to provide polychromate-based baths with high covering-power which produce penetrating and bright deposits, are easily used on an industrial scale and have high cathode efficiencies.

This object is achieved by the present invention, which relates to a process for chromium-plating by electrodeposition of chromium from a bath comprising polychromates and sulphates, characterized by effecting the said electrodeposition in the presence of sulphonamides of formula R-SO₂Y, where R is an alkyl chain and Y is an amine group, and in which the ratio of carbon atoms in the R chain and nitrogen atoms in the amino group Y is < 12, or of the corresponding sulphonimides.

The invention also relates to a chromate bath for the realization of the above process.

It was further discovered, surprisingly, that sulphonamides, or the corresponding sulphonimides, added to a chromium bath comprising polychromates and sulphates had an unexpected protective effect on the anode of the same.

The use of sulphonamides or sulphonimides to protect the anode of a chromium bath is therefore a further object of the invention.

According to a preferential embodiment of the invention, the sulphonamide used has the general formula R-SO₂-NR'R", where R is a linear alkyl chain C1-C12, R' and R" are, together or separately, hydrogen, -NH₂, -NHOH, -CONH₂ or an aliphatic or heterocyclic substituent.

According to another aspect of the invention Na, Mg or ammonium salts of alkyl sulphonic acids of the general formula R-SO₃-, where the ratio between the sulphur atoms and the carbon atoms in the R chain is greater or equal to 1/4, (S:C ≥ 1:4), or corresponding salts of sulfamic acid, are used to increase the covering power of the bath and to give extensive substantially uniform micro-cracking in the presence of selenium.

Further objects of the invention are therefore the use of salts of alkyl sulphonic acids according to Claim 12 and the use of salts of sulfamic acid according to Claim 13.

The invention has numerous advantages over the present state of the art. The use of sulphonamides or sulphonimides gives bright deposits; the use of polychromates in the salt form results in stable baths even if bath temperature is changed; the sulphonamides protect the anodes from corrosion; the use of Na, Mg or NH₄⁺ cations (obtained from their corresponding salts of the alkyl sulphonic acids or sulfamic acid) increases the covering power and gives extensive substantially uniform micro-cracking in the presence of selenium.

### Best Mode for Carrying Out the Invention

Preferred polychromates are tri- and tetra-chromates as well as higher homologues. These compounds are obtained by treating their corresponding di-chromates with nitric acid or chromic anhydride.

The following is a list (which is illustrative but not limiting) of polychromates according to the invention:

| Compound | Method of production |
|---|---|
| (NH₄)₂Cr₃O₁₀ | (NH₄)₂Cr₂O₇ + HNO₃ |
| K₂Cr₃O₁₀ | K₂Cr₂O₇ + HNO₃ |
| MgCr₄O₁₃ | MgCO₃ + CrO₃ |
| (NH₄)₂Cr₄O₁₃ | (NH₄)₂Cr₂O₇ + HNO₃ |
| K₂Cr₄O₁₃ | K₂Cr₃O₁₀ + HNO₃ |
| SrCr₃O₁₀ | SrCr₂O₇ + CrO₃ |

Some of these compounds were obtained in the presence of chromium borate as initiator. The preferred concentration of such compound in the bath was between 4 and 40 g/litre. These polychromates, in aqueous solution with a preferred concentration of between 200 and 400 g/l, give a bath which is unaffected by changes in temperature and which maintains a high cathode efficiency even with relatively high temperatures. The preferred operating temperature is between 40 and 70°C and more preferably, between 45 and 60°C. The ratio of polychromate concentration to sulphate concentration is preferably between 20 and 250.

The deposits obtained from these baths are dull and have low covering power. It was surprising to find that bright deposits can be obtained if sulphonamides of the type R-SO₃-NH₂ (where R is a linear alkyl chain C1-C12) or the corresponding sulphonimides are added to the bath.

When sulphonamides or the corresponding sulphonimides are added to the polychromate bath, the crystalline structure of the chromium deposit is modified from large-grain hexagonal (dull deposit) to fine-grain body-centered cubic structure (bright deposit).

Short-chain alkyl sulphonic acids have been used as additives in some of the known electroplating processes to increase the cathode efficiency of the bath (in chromic acid based baths) as described, for instance, in EP-A-0196053. However, the alkyl sulphonic acids have the disadvantage of causing electrochemical corrosion of anodes in Pb/Sn and in other lead-based alloys. This corrosion occurs both in the chromic acid based chromium baths and in polychromate based baths as in the present invention, though in the latter it is in a reduced form due to the less acid pH of the same.

As described above, it has been discovered that the presence of sulphonamides or sulphonimides of the type already described confer high resistance to corrosion of the anode by the alkyl sulphonic acids in the chromium plating baths.

The sulphonamides and the sulphonimides have the same function in protecting the anode even in traditional baths based on chromic acid and sulphuric acid. The use of sulphonamides and sulphonimides in such traditional baths has been found to have other advantages, in particular, to lead to higher cathode efficiency and brighter deposits. A further object of the invention is thus the use of sulphonamides or sulphonimides according to Claim 14.

The sulphonamides preferably used in the present invention are generally prepared by the Schotten and Baumann reaction of chlorides of C1-C12 alkyl sulphonic acids: ${\text{R-SO}}_{\text{2}} {\text{Cl + NH}}_{\text{3}} {\text{+ NaOH → R-SO}}_{\text{2}} {\text{NH}}_{\text{2}} {\text{+ NaCl + H}}_{\text{2}} \text{O}$Ammonium compounds such as hydroxylamine, hydrazine, urea, aliphatic or heterocyclic amines may be used instead of ammonia.

The aliphatic amines are preferably primary amines with aliphatic C1-C12 chain.

The sulphonamides of interest for the present invention are those mentioned above with the general formula R-SO₂-NR'R", where R is a C1-C12 alkyl chain and R' and R" are, together or separately, hydrogen, -NH₂, -NHOH, -CONH₂ or an aliphatic or heterocyclic substituent.

Preferred concentrations of sulphonamides are such as to give a ratio of the concentration (by weight) of polychromate to the concentration (by weight) of sulphonamide of between 20 and 450.

It has been found that the covering power of the chromium deposits obtained from a chromium bath is improved by the addition of Na⁺, Mg²⁺ and ammonium ions.

Such ions are present (either alone or in combination) in total concentrations of from 2 to 30 g/l in addition to any such cations that are possibly present in the polychromates used.

These cations are preferably added to the bath in the form of contra-ions of the organic anions of alkyl sulphonic acids R-SO₃H, where R is a C1-C4 alkyl group with possible substitution in the 2 position by -OH or -NH2. Preferred salts are Na, Mg or ammonium salts of CH₃SO₃⁻; CH₃CH₂SO₃⁻; CH₃CH₂CH₂SO₃⁻; CH₃CH(OH)CH₂SO₃⁻; NH₂CH₂CH₂SO₃⁻.

The corresponding salts of sulphamic acid, i.e. NH₂SO₃Na; (NH₂SO₃)₂Mg; NH₂SO₃NH₄ can also be used. These compounds are chosen as sources of cations because they do change neither the internal equilibrium of the polychromate nor the polychromate/sulphate ratio, which would change if the sulphate of the chosen cation was used.

The preferred concentration of the alkylsulphonic salts are those which gives a ratio of polychromate concentration (by weight) to alkyl sulphonic acids concentration (by weight) between 25 and 450.

A further advantage of using the cations referred to above is that they produce very extensive micro-cracking in the presence of selenium even in areas of reduced current density.

The process according to the invention provides, having prepared a bath giving the characteristics listed above, for operation at a current density of between 11 and 230 A/dm² and preferably between 30 and 100 A/dm².

In conclusion, the bath according to the present invention produces a bright, adhering and non-iridescent deposit on a metal base, free of grey or rough deposit at low current-density with a cathode efficiency of at least 25% measured at a current density of 50 A/dm² and a chromate bath temperature of 52°C.

The invention will now be further described with reference to examples which are illustrative but not limiting.

### Example 1.

A chromate bath was prepared, based on tri- and tetra-chromates with the following initial composition :

| | |
|---|---|
| Polychromate | 380 g/l |
| H₂SO₄ | 3.5 g/l |

A Standard Hull Cell was used to produce chromium-plating; the cathode efficiency was 25%, with a dull deposit.

### Example 2.

Sulphonamides were added to the bath of Example 1 in a series of steps to give from 2 g/l to 12 g/l. The sulphonamides tested had R= linear alkyl with 1, 4, 6, 10 and 12 carbon atoms.

The cathode efficiency was still 25%. The deposit was bright in all concentrations of the example.

### Example 3

Sodium cation bound to alkyl sulphonic acid as a salt was added to the bath of Example 2 in increasing quantities. The cathode used in this bath was a 1.5 X 15 cm "V"-shaped panel.

The chromium plating was carried out at a current of 10 A. The distance of the plating from the base of the indentation was the following:

| Sodium Alkyl Sulphonate (g/l) | Non-plated (mm) |
|---|---|
| 0 | 8.5 |
| 2 | 4.0 |
| 4 | 3.0 |
| 10 | 2.0 |
| 20 | 0.0 |

## Claims

1. A process for chromium-plating by electrodeposition of chromium from a bath comprising polychromates and sulphates, characterized by effecting the said electrodeposition in the presence of sulphonamides of formula R-SO₂Y, where R is an alkyl chain and Y is an amine group, and in which the ratio of carbon atoms in the R chain and nitrogen atoms in the amino group is less or equal to twelve (C/N 12), or in the presence of the corresponding sulphonimides.

2. A process according to claim 1, characterized by operating in the presence of Mg, Na or ammonium ions or a mixture thereof.

3. A process according to claim 2, characterized by adding at least a part of the said ions to the said chromium-plating bath in the form of the corresponding salts of alkyl sulphonic acids of formula R-SO₃⁻, where R is an alkyl chain and where the ratio between the sulphur atoms and the carbon atoms of the R chain is greater or equal to 1/4, (S:C ≥ 1:4), or salts of sulphamic acid or salts of C2-C4 alkyl sulphonic acids substituted in position 2.

4. A process according to any of the claims 1 to 3, characterized by operating in the presence of sulphonamides with formula R-SO₂-NR'R", where R is a linear C1-C12 alkyl group and R' and R" are, together or separately, hydrogen, -NH₂, -NHOH, -CONH₂ or an aliphatic or heterocyclic substituent, or in the presence of the corresponding sulphonimides.

5. A process according to claim 3 or 4, wherein the concentration of polychromates is within the range from 200 to 400 g/l.

6. A process according to any previous claim, wherein the ratio between the concentration of the said polychromates and the concentration of the sulphonamides is within the range from 20 to 450.

7. A process according to claim 3 and claim 5 or 6, wherein the ratio between the concentration of the said polychromates and the concentration of the salts of Na, Mg and ammonium is within the range from 20 to 450.

8. A process according to any of the preceding claims, wherein the bath temperature is within the range of 45 to 65°C.

9. A chromium-plating bath for the electrodeposition of chromium from a solution of polychromates, characterized by having a composition according to any of the claims 1 to 8.

10. The use of sulphonamides of formula R-SO₂-Y, where R is an alkyl chain, Y is an amino group and in which the ratio of carbon atoms in the R chain and nitrogen atoms in the amino group Y is ≤ 12 (C/N≤12), or of the corresponding sulphonimides in a chromium-plating bath comprising polychromates and sulphates to obtain bright chromium deposits.

11. The use of sulphonamides according to Claim 10, or of the corresponding sulphonimides, in a chromium-plating bath comprising polychromates and sulphates to protect the anode of the said bath.

12. The use of alkyl sulphonic salts of formula (R(R')SO₃)ₙX where R is a C1-C4 alkyl group, R' is H, NH₂ or OH in position 2 of the R group, X is a cation selected from Na, Mg or NH₄⁺ and where n = 2 when X is Mg but n = 1 otherwise, to increase the covering power in a chromium-plating bath comprising polychromates and sulphates.

13. The use of salts of Na, Mg or NH₄ of sulphamic acid, or a mixture thereof, to increase covering power in a chromium-plating bath comprising polychromates and sulphates.

14. The use of sulphonamides or sulphonimides in a chromium-plating bath comprising chromic acid and sulphuric acid to improve the brightness of chromium deposit and the cathode efficiency, and to protect the anode of the said bath.

## Patentansprüche

1. Verfahren zum Verchromen durch elektrolytisches Abscheiden von Chrom aus einem Polychromate und Sulfate enthaltenden Bad, gekennzeichnet durch Bewirken der elektrolytischen Abscheidung in Anwesenheit von Sulfonamiden der Formel R-SO₂Y, worin R eine Alkylkette und Y eine Aminogruppe ist und in der das Verhältnis der Kohlenstoffatome in der R-Kette und Stickstoffatome in der Aminogruppe kleiner oder gleich zwölf ist (C/N ≤ 12), oder in Anwesenheit von entsprechenden Sulfonimiden.

2. Verfahren gemäß Anspruch 1, gekennzeichnet durch Arbeiten in Anwesenheit von Mg-, Na- oder Ammoniumionen oder einer Mischung daraus.

3. Verfahren gemäß Anspruch 2, gekennzeichnet durch Zufügen mindestens eines Teiles der Ionen zu dem Verchromungsbad in Form der entsprechenden Salze der Alkylsulfonsäuren der Formel R-SO₃⁻, worin R eine Alkylkette ist und das Verhältnis zwischen den Schwefelatomen und den Kohlenstoffatomen der R-Kette größer oder gleich 1/4 ist (S:C ≥ 1:4), oder Salzen der Sulfaminsäure oder Salzen der in Position 2 ersetzten C₂-C₄-Alkylsulfonsäuren.

4. Verfahren gemäß einem der Ansprüche 1 -3, gekennzeichnet durch Arbeiten in Anwesenheit von Sulfonamiden mit der Formel R-SO₂-NR'R", worin R eine lineare C₁-C₁₂-Alkylgruppe und R' und R", zusammen oder getrennt, Wasserstoff, -NH₂, -NHOH, -CONH₂ oder ein aliphatischer oder heterozyklischer Substituent sind, oder in Anwesenheit entsprechender Sulfonimide.

5. Verfahren gemäß Anspruch 3 oder 4, bei dem die Konzentration der Polychromate im Bereich von 200 bis 400 g/l liegt.

6. Verfahren gemäß einem der vorhergehenden Ansprüche, bei dem das Verhältnis zwischen der Konzentration der Polychromate und der Konzentration der Sulfonamide im Bereich von 20 bis 450 liegt.

7. Verfahren gemäß Anspruch 3 und Anspruch 5 oder 6, bei dem das Verhältnis zwischen der Konzentration der Polychromate und der Konzentration der Na-, Mg- und Ammonium-Salze im Bereich von 20 bis 450 liegt.

8. Verfahren gemäß einem der vorhergehenden Ansprüche, bei dem die Badtemperatur im Bereich von 45 bis 65 °C liegt.

9. Verchromungsbad für die elektrolytische Abscheidung von Chrom aus einer Lösung aus Polychromaten, gekennzeichnet durch eine Zusammensetzung gemäß einem der Ansprüche 1 - 8.

10. Anwendung von Sulfonamiden der Formel R-SO₂-Y, worin R eine Alkylkette, Y eine Aminogruppe und in der das Verhältnis der Kohlenstoffatome in der R-Kette und der Stickstoffatome in der Aminogruppe Y ≤ 12 ist (C/N ≤ 12), oder der entsprechenden Sulfonimide in einem Polychromate und Sulfate enthaltenden Verchromungsbad zum Erhalten hochglänzender Verchromungen.

11. Anwendung von Sulfonamiden gemäß Anspruch 10, oder der entsprechenden Sulfonimide, in einem Verchromungsbad, das Polychromate und Sulfate zum Schutz der Anode des Bades enthält.

12. Anwendung von Alkylsulfonsalzen der Formel (R(R')SO₃)ₙX, worin R eine C₁-C₄-Alkylgruppe ist, R' in Position 2 der R-Gruppe H, NH₂ oder OH ist, X ein aus Na, Mg oder NH₄⁺ ausgewähltes Kation ist und worin n = 2 ist, wenn X Mg ist, jedoch ansonsten n = 1 ist, um die Deckkraft in einem Polychromate und Sulfate enthaltenden Verchromungsbad zu erhöhen.

13. Anwendung von Na-, Mg- oder NH₄-Salzen der Sulfaminsäure oder einer Mischung daraus zum Erhöhen der Deckkraft in einem Polychromate und Sulfate enthaltenden Verchromungsbad.

14. Anwendung von Sulfonamiden oder Sulfonimiden in einem Chromsäure und Schwefelsäure enthaltenden Verchromungsbad zum Verbessern des Glanzes des Chromauftrages und der katodischen Stromausbeute und zum Schutz der Anode des Bades.

## Revendications

1. Procédé pour le chromage par dépôt électrolytique de chrome à partir d'un bain comprenant des polychromates et des sulfates, caractérisé par la réalisation du dit dépôt électrolytique en présence de sulfonamides de formule R-SO₂Y, dans laquelle R est une chaîne alkyle et Y est un groupe amine, et où le rapport des atomes de carbone dans la chaîne R et des atomes d'azote dans le groupe amino Y est inférieur ou égal à 12 (C/N ≤ 12), ou en présence des sulfonimides correspondants.

2. Procédé suivant la revendication 1, caractérisé par le fonctionnement en présence d'ions Mg, Na ou ammonium ou d'un mélange de ceux-ci.

3. Procédé suivant la revendication 2, caractérisé par l'addition d'au moins une partie des dits ions audit bain de chromage sous la forme des sels correspondants d'acides alkyl sulfoniques de formule générale R-SO₃⁻, dans laquelle R est une chaîne alkyle et où le rapport entre les atomes de soufre et les atomes de carbone de la chaîne R est supérieur ou égal à 1/4, (S:C ≥ 1:4), ou des sels d'acide sulfamique ou des sels d'acides alkyl sulfoniques en C₂₋₄ substitués en position 2.

4. Procédé suivant l'une quelconque des revendications 1 à 3, caractérisé par le fonctionnement en présence de sulfonamides ayant la formule générale R-SO₂-NR'R", dans laquelle R est une chaîne alkyle linéaire en C₁₋₁₂, R' et R" sont, ensemble ou séparément, un atome d'hydrogène, un groupe -NH₂, -NHOH, -CONH₂ ou un substituant aliphatique ou hétérocyclique, ou en présence des sulfonimides correspondants.

5. Procédé suivant les revendications 3 ou 4, dans lequel la concentration des polychromates est comprise dans la gamme de 200 à 400 g/l.

6. Procédé suivant l'une quelconque des revendications précédentes, dans lequel le rapport entre la concentration des dits polychromates et la concentration des sulfonamides est comprise dans la gamme de 20 à 450.

7. Procédé suivant la revendication 3 et les revendications 5 ou 6, dans lequel le rapport entre la concentration des dits polychromates et la concentration des sels de Na, de Mg et d'ammonium est comprise dans la gamme de 20 à 450.

8. Procédé suivant l'une quelconque des revendications précédentes, dans lequel la température du bain est comprise dans la gamme de 45°C à 65°C.

9. Bain de chromage pour le dépôt électrolytique de chrome à partir d'une solution de polychromates, caractérisé en ce qu'il a une composition suivant l'une quelconque des revendications 1 à 8.

10. Utilisation de sulfonamides de formule R-SO₂Y, dans laquelle R est une chaîne alkyle, Y est un groupe amino, et où le rapport des atomes de carbone dans la chaîne R et des atomes d'azote dans le groupe amino Y est inférieur ou égal à 12 (C/N ≤ 12), ou des sulfonimides correspondants dans un bain de chromage comprenant des polychromates et des sulfates pour obtenir des dépôts de chrome brillants.

11. Utilisation de sulfonamides suivant la revendication 10, ou des sulfonimides correspondants, dans un bain de chromage comprenant des polychromates et des sulfates pour protéger l'anode du dit bain.

12. Utilisation de sels alkyl sulfoniques de formule [R(R')SO₃]ₙX dans laquelle R est un groupe alkyle en C₁₋₄, R' est un atome d'hydrogène, un groupe NH₂ ou OH en position 2 du groupe R, X est un cation choisi parmi Na, Mg ou NH₄⁺ et où n = 2 lorsque X est Mg, mais n = 1 dans les autres cas, pour augmenter le pouvoir couvrant dans un bain de chromage comprenant des polychromates et des sulfates.

13. Utilisation des sels de Na, de Mg ou de NH₄ d'acide sulfamique, ou d'un mélange de ceux-ci, pour augmenter le pouvoir couvrant dans un bain de chromage comprenant des polychromates et des sulfates.

14. Utilisation de sulfonamides ou de sulfonimides dans un bain de chromage comprenant de l'acide chromique et de l'acide sulfurique pour améliorer le brillant du dépôt de chrome et le rendement cathodique, et pour protéger l'anode du dit bain.
